

corporated into 99.5 g. of the polyethylene. The results are shown in the following table:

TABLE 6

| Antistatic agent                            | Surface resistance, ohms | Static charge, volts |
|---------------------------------------------|--------------------------|----------------------|
| "D-Stat B"                                  | $1 \times 10^{11}$       | 400                  |
| "Nopcone LV"                                | $1.5 \times 10^{13}$     | 800                  |
| "Merix Anti-Static 79 OL"                   | $5 \times 10^{13}$       | 500                  |
| "Statikil"                                  | $2 \times 10^{13}$       | 200                  |
| "Plexiklar"                                 | $5 \times 10^{13}$       | 500                  |
| <chem>C11H23-C(=O)-NH-(CH2)3-N(CH3)2</chem> | $1 \times 10^9$          | 0                    |

## EXAMPLE 7

In another series of comparative tests, there was used a commercial, granulated polypropylene sold under the name "Luparen 151 white," this polymer having an intrinsic viscosity of 2.8, a mean molecular weight of 500,000 and a density of 0.905 g./cm.<sup>3</sup>.

In each test, 0.1 g. of the antistatic agent as listed in Table 7 were incorporated into 99.9 g. of the polypropylene. The substances were mixed on a conventional rolling mill for five minutes at 175° C. The rolled sheet obtained thereby was cooled to 20° C. and then subjected to a pressure of 180 atm. at 175° C. for two minutes in a press and pressed into sheets 10 cm. square and 2 mm. thick. These sheets were stored for three days at 20° C. in a cabinet maintained at an atmospheric humidity of 46%. The surface resistance and static charge were then determined as in the preceding two examples with the following results:

TABLE 7

| Antistatic agent                            | Surface resistance, ohms | Static charge, volts |
|---------------------------------------------|--------------------------|----------------------|
| "D-Stat B"                                  | $2 \times 10^{13}$       | 600                  |
| "Nopcone LV"                                | $2 \times 10^{13}$       | 400                  |
| "Merix Anti-Static 79 OL"                   | $5 \times 10^{14}$       | 200                  |
| "Statikil"                                  | $1 \times 10^{14}$       | 400                  |
| "Plexiklar"                                 | $2 \times 10^{14}$       | 900                  |
| <chem>C11H23-C(=O)-NH-(CH2)3-N(CH3)2</chem> | $1 \times 10^{10}$       | 20                   |

## EXAMPLE 8

The same procedure and materials were used as in Example 7 except that 0.5 g. of the antistatic agent were incorporated into 99.5 g. of the polypropylene. The following results were obtained:

TABLE 8

| Antistatic agent                            | Surface resistance, ohms | Static charge, volts |
|---------------------------------------------|--------------------------|----------------------|
| "D-Stat B"                                  | $1 \times 10^{13}$       | 400                  |
| "Nopcone LV"                                | $2 \times 10^{13}$       | 100                  |
| "Merix Anti-Static 79 OL"                   | $5 \times 10^{13}$       | 100                  |
| "Statikil"                                  | $2 \times 10^{13}$       | 400                  |
| "Plexiklar"                                 | $2 \times 10^{13}$       | 350                  |
| <chem>C11H23-C(=O)-NH-(CH2)3-N(CH3)2</chem> | $5 \times 10^9$          | 0                    |

It will be readily apparent from these series of comparative tests that antistatic agents commonly used for the surface treatment of various thermoplastic material do not give the same effective results as the particular antistatic agent of the present invention when incorporated or blended into polyethylene or polypropylene as a molding material. Surprisingly, the amine compounds em-

ployed herein do give excellent results under these conditions even when used in amounts of less than 1% by weight with reference to the polymonoolefin.

The invention is hereby claimed as follows:

5 1. A thermoplastic composition comprising a polymonoolefin containing dispersed therein as an antistatic additive about 0.01 to 5% by weight of a compound of the formula



15 in which  $\text{R}_1$  denotes a hydrocarbon radical selected from the class consisting of alkyl and alkenyl of 1 to 40 carbon atoms,  $\text{R}_2$  and  $\text{R}_3$  each denotes lower alkyl of 1 to 4 carbon atoms,  $\text{R}_4$  denotes alkylene of 1 to 10 carbon atoms and  $\text{X}$  denotes a divalent radical selected from the class consisting of  $-\text{O}-$  and  $-\text{NH}-$ .

20 2. A composition as claimed in claim 1 wherein said antistatic additive is present in an amount of about 0.1 to 2% by weight with reference to the polymonoolefin.

25 3. A composition as claimed in claim 1 wherein the polymonoolefin is a polymer selected from the class consisting of polyethylene, polypropylene and mixtures thereof.

4. A composition as claimed in claim 1 wherein the antistatic agent is a compound of the formula



35 in which  $\text{R}_1$  denotes a hydrocarbon radical selected from the class consisting of alkyl and alkenyl of 3 to 20 carbon atoms,  $\text{R}_2$  and  $\text{R}_3$  each denotes lower alkyl of 1 to 4 carbon atoms,  $\text{R}_4$  denotes alkylene of 2 to 6 carbon atoms and  $\text{X}$  denotes a divalent radical selected from the class consisting of  $-\text{O}-$  and  $-\text{NH}-$ .

40 5. A composition as claimed in claim 1 wherein said antistatic additive is N-lauroyl-N'-dimethyltrimethylene diamine.

45 6. A composition as claimed in claim 5 wherein said polymonoolefin is a polymer selected from the class consisting of polyethylene, polypropylene and mixtures thereof.

7. A composition as claimed in claim 6 wherein said antistatic additive is present in an amount of about 0.1 to 2% by weight with reference to the polymonoolefin.

50 8. A composition as claimed in claim 6 wherein said polymonoolefin has a molecular weight between 20,000 and 1,000,000, the polyethylene having a density between 0.94 and 0.97 g./cm.<sup>3</sup> and the polypropylene having a density between 0.890 and 0.910 g./cm.<sup>3</sup>.

## References Cited

## UNITED STATES PATENTS

|           |         |                       |           |
|-----------|---------|-----------------------|-----------|
| 2,921,048 | 1/1960  | Bell et al. -----     | 260—45.9  |
| 2,525,691 | 10/1950 | Lee et al. -----      | 260—31.4  |
| 3,190,763 | 6/1965  | Schleepe et al. ----- | 106—186   |
| 2,403,960 | 7/1946  | Stoops et al. -----   | 117—139.5 |
| 3,211,646 | 10/1965 | Berger -----          | 252—8.8   |

JOSEPH L. SCHOFER, Primary Examiner

S. M. LEVIN, Assistant Examiner

U.S. Cl. X.R.

65 260—93.7, 94.9







In this example, two PTHF materials are employed, one having an intrinsic viscosity of 3.8 (dl./gm.) and the other 16. The milled sheets are preheated 5 minutes at 350° F. and then molded 3 minutes at 350° F. under 30,000 lbs. pressure in a standard ASTM tensile sheet mold. The material is allowed to cool to R.T. under full pressure. The resulting sheets are tested for their physical properties. The data are as follows:

| Material                  | Sample No.—parts/wt. |      |      |       |       |      |
|---------------------------|----------------------|------|------|-------|-------|------|
|                           | A                    | B    | C    | D     | E     | F    |
| PVC batch (above)         | 84.75                |      |      |       |       |      |
| PTHF ( $\eta=16$ )        | 3.75                 | 7.5  | 15.0 |       |       |      |
| PTHF ( $\eta=3.8$ )       |                      |      |      | 3.75  | 7.5   | 15.0 |
| HDT (264 p.s.i.) °C       | 69                   | 68   | 67.5 | 69.5  | 68    | 65   |
| Notched Izod ft. lbs./in. | 2.48                 | 8.87 | 2.19 | 15.74 | 10.32 | 8.15 |

During the preparation of these blends, samples D through F exhibited quite good processing behavior and formed very smooth molded sheets. Sample C exhibited the poorest processing behavior.

Excess material from sample C above is remilled for various times at various temperatures up to 400° F. At 380° F. the material banded quite well and the smoothness of the "bank" at the nip of the rolls improved with best milling behavior being obtained at 400° F. The portion milled at 400° F. is press molded as described at 410° F. to form tensile sheets which exhibit an average Notched Izod impact (4 sheets) of 16.48 ft. lbs./in. It appears that the higher molecular weight PTHF requires higher processing temperatures but forms blends of excellent impact resistance. The latter experiment indicates most clearly the great thermal stability of these blends since the total heat history of the sample exhibiting 16.48 ft. lbs./in. Izod impact is quite considerable.

### EXAMPLE III

In this example, a PTHF made as described in Example I, having an  $[\eta]$  of 7.57 is employed in blends with the same polyvinyl chloride base resin. In this case the two resins are combined in a container with a fairly large quantity of monomeric THF and rolled on a paint roller until dissolved. The resulting solution is poured into water to precipitate the polymer content and the resulting solid blended material dried overnight in a vacuum oven at 50° C. The dried material in each case is milled to form sheets. The resulting sheets are press molded by the procedure described at 350° F. and the resulting molded sheets subjected to a proprietary dynamic extrusion test employing a constant load rheometer. In this test a quantity of the blend is confined in an orifice-equipped cylinder (orifice  $d=0.0459$  inch and  $l=0.3260$  inch) under a piston exerting a constant 400 p.s.i. pressure and the assembly gradually heated while noting and recording the movement of the piston. The temperature at which the piston stops its downward movement ( $T_1$ ) occurs is the point of full compacting of the plastic and is related to the second order transition temperature. On continued heating beyond the  $T_1$  value, a temperature is reached where the piston again moves downwardly accompanied by extrusion of the plastic through the orifice. The temperature ( $T_2$ ) at which the latter begins is the melt flow point. The  $T_1/T_2$  values thus determined together with Instron tensile and elongation values, Shore A Hardness, and tensile impact values (expressed in ft. lbs./in. of thickness) also are listed below.

The above data indicate no pronounced advantage in a molecular weight intermediate the 3.8 and 16 values of intrinsic viscosity. However, the data is interesting since the ultimate tensile seems to be high at low PTHF levels, then goes through a minimum in the region of about 25 parts/wt. of PTHF per 100 parts/wt. of PVC and then rise sharply at the 50/50 point of concentration. The extremely high impact values above the PTHF level of about 20 parts/wt. per 100 parts/wt. of PVC indicate a loss of rigidity. Visual examination confirms this since the samples 1 and 2 definitely are more pliable than is sample 4 (10 PHR level).

The above data indicate that the addition of PTHF depresses both the  $T_1$  and  $T_2$  values of the base resin almost linearly with concentration above the point of 10 parts/wt. of PTHF per 100 parts/wt. of polyvinyl chloride. Compare the relatively small effect on the HDT values shown in Example II at levels of PTHF below 10 parts/wt. per 100 parts/wt. of the base resin.

20 The above data, it should be noted, is obtained on formulations containing no added compounding ingredients.

### EXAMPLE IV

The stability of the blends of this invention is again evaluated by a standard accelerated air oven aging at 350° F. In this example all blends are prepared by milling 5 minutes at 350° F. In this examination several types of control formulations are employed for purposes of comparison. One such type of control is a conventional non-rigid polyvinyl chloride compound plasticized with up to 50 PHR of diethyl phthalate compound and the other type is a conventional high-impact rigid polyvinyl chloride employing, as an impact improver, 10 PHR on the polyvinyl chloride of a styrene/acrylonitrile copolymer on polybutadiene known as "Hycar 1010 X 43" made by the B.F. Goodrich Chemical Company, of Akron, Ohio. In the latter experiment, the PVC/1010 X 43 type control blend definitely begins to yellow in the range of from about 120 to about 150 minutes at 350° F. wherein the experimental blend containing 10 PHR of PTHF  $[\eta]=3.8$  is not as yellow after as much as 370 minutes as is the PVC/1010 X 43 control at 150 minutes. At the end (920 minutes at 350° F.) of the even aging test, the PVC/1010 X 43 control blend is completely black whereas the experimental PTHF blend is only a mustard color or light brown. In the other series of experiments, the blends (prepared by the solution blending technique of Example III) containing various PTHF materials ( $\eta=3.8$ ; 7.6 and 16) containing no stabilizer are compared to unstabilized plasticized (diethyl phthalate) compounds of the same polyvinyl chloride. Blends containing 10 to 50 PHR of PTHF are slightly better in heat resistance than the controls of corresponding diethyl phthalate content. While the differences are small, it seems that the samples of blends containing the PTHF of intrinsic viscosity 7.6 are slightly more stable and retained their shape better than the corresponding blends containing PTHF of higher and lower molecular weight.

### EXAMPLE V

In this example, the preparation of several cross-linked or partially-gelled PTHF materials is described. In each case, about 200 grams of the solid, dry PTHF is dissolved in about 2400 ml. of benzene. To each of the resulting solutions, about 8 grams of dicumyl peroxide and 1.2 grams of sulfur are added and the solution

| Sample No. | Wt. PTHF, gms. | Wt. PVC, gms. | $T_1$ , °C. | $T_2$ , °C. | Tensile, p.s.i. | Elong. | Shore "A" | Tensile impact, ft. lbs./in. |
|------------|----------------|---------------|-------------|-------------|-----------------|--------|-----------|------------------------------|
| 1.         | 15             | 15            | 35          | 101         | 5,512           | 430    | 97        | 40.21                        |
| 2.         | 10             | 20            | 53          | 111         | 4,444           | 290    | 98        | 31.63                        |
| 3.         | 6              | 24            | 66          | 108         | 3,891           | 80     | 98        | 13.42                        |
| 4.         | 3              | 30            | 80          | 130         | 6,390           | 50     | 96        | 15.22                        |
| 5.         |                | 30            | 86          | 138         | 7,386           | 60     | 95        | 8.04                         |
| 6.         | 130            | -15           | +85         |             | 6,000           | 600    | 296       |                              |

<sup>1</sup> I.V. 3.8. <sup>2</sup> Crystalline-form.

## 11

thoroughly mixed at room temperature to dissolve the peroxide and distribute the additives throughout the mix. The benzene content of each solution is then evaporated off at 50° C. under vacuum. The resulting rubbery material is then placed in a mold under pressure and heated at 150° C. for about 3 hours to induce the cross-linking reaction. Each of the molded materials, each weighing about 210 grams, is placed under Dry Ice to bring about recrystallization (although the same would occur on standing for some time at room temperature). Each molded specimen is tested for gel content by a Soxhlet-type "sol-gel" extraction procedure employing 50-mesh wire filter screens and boiling ethyl acetate. The data are as follows:

| X-PTHF           |                               |                    |
|------------------|-------------------------------|--------------------|
| Parent PTHF=1.11 |                               |                    |
|                  | P.h.r.<br>dicumyl<br>peroxide | Percent/wt.<br>gel |
| Sample No.:      |                               |                    |
| 1-----           | 0                             | 0                  |
| 2-----           | 4                             | 79.6               |
| 3-----           | 6                             | 6.6                |
| X-PTHF           |                               |                    |
| Parent PTHF=3.8  |                               |                    |
|                  |                               |                    |
| 4-----           | 0                             | 0                  |
| 5-----           | 2                             | 58.9               |
| 6-----           | 4                             | 89.0               |

## EXAMPLE VI

The X-PTHF materials of the foregoing example are combined with polyvinyl chloride ( $\eta=0.94$  by method described above under Vinyl Chloride Resin) each blend containing 10 PHR of X-PTHF. The blends are made using the masterbatch recipe and procedure of Example II and are each prepared by mill-mixing for various in-

| Sample No. | Polyvinyl chloride base resin parts/wt. | Lubricant                  |           | TiO <sub>2</sub> parts/wt. | Type                             | Processing aid | Stabilizer* parts/wt. | Izod, ft./lbs./in. | Notes            |
|------------|-----------------------------------------|----------------------------|-----------|----------------------------|----------------------------------|----------------|-----------------------|--------------------|------------------|
|            |                                         | Type                       | Parts/wt. |                            |                                  |                |                       |                    |                  |
| 909A-----  | 100                                     | Cadmium stearate           | 2         | 5                          | Styrene-acrylonitrile copolymer. | 3              | 3                     | 10                 | 12.25 Good bank. |
| 909B-----  | 100                                     | do                         | 2         | 5                          | Polyethylene <sup>1</sup>        | 1.0            | 3                     | 10                 | 15.56 Do.        |
| 909C-----  | 100                                     | do                         | 2         | 5                          | Polypropylene <sup>2</sup>       | 1.0            | 3                     | 10                 | 16.27 Do.        |
| 909D-----  | 100                                     | Polyethylene <sup>1</sup>  | 1.0       | 5                          | Same as A                        | 3              | 3                     | 10                 | 4.82 Do.         |
| 909E-----  | 100                                     | Polypropylene <sup>2</sup> | 1.0       | 5                          | do                               | 3              | 3                     | 10                 | 9.10 Do.         |
| 909F-----  | 100                                     | Same as A                  | 2         | 5                          | None                             | 3              | 10                    | 1.61               |                  |

\* Dibutyl tin thioglycolate.

<sup>1</sup> Low molecular weight polyethylene, "AC 629 A" made by Allied

dictated times at various temperatures from 335 to 440° F. The data are as follows:

| PVC/X-PTHF BLENDS                 |            |            |                                                |  |
|-----------------------------------|------------|------------|------------------------------------------------|--|
| X-PTHF (Parent PTHF, $\eta=1.1$ ) |            |            |                                                |  |
| Percent gel                       | Milling    |            | Notched Izod input strength (ft.lbs./in notch) |  |
|                                   | Temp., °C. | Time, min. | (ft.lbs./in notch)                             |  |
| 0-----                            | 380        | 5          | 1.5                                            |  |
| 79.6-----                         | 380        | 5          | 10.0                                           |  |
| 86.6-----                         | 380        | 5          | 1.13                                           |  |

| PVC/X-PTHF BLENDS                 |            |                                              |         |         |         |
|-----------------------------------|------------|----------------------------------------------|---------|---------|---------|
| X-PTHF (Parent PTHF, $\eta=3.8$ ) |            |                                              |         |         |         |
| Percent gel                       | Temp., °C. | Izod vs. time of milling (ft./lbs./in notch) |         |         |         |
|                                   |            | 5 min.                                       | 10 min. | 20 min. | 30 min. |
| 0 (control)-----                  | 335        | 13.62                                        | 13.41   | 8.34    | 9.94    |
| 0 (control)-----                  | 380        | 13.86                                        | 12.09   | 13.05   | 4.61    |
| 0 (control)-----                  | 410        | 11.90                                        | 11.73   | 1.58    | 0.66    |
| 0 (control)-----                  | 440        | 6.01                                         | 1.68    | N.d.    | N.d.    |
| 58.9-----                         | 335        | 1.38                                         | 2.67    | 14.47   | 15.07   |
| 58.9-----                         | 380        | 11.00                                        | 10.55   | 13.00   | 10.66   |
| 58.9-----                         | 410        | 9.48                                         | 11.12   | 1.76    | N.d.    |
| 58.9-----                         | 440        | 10.31                                        | 12.66   | N.d.    | N.d.    |
| 80.8-----                         | 335        | 0.57                                         | 0.64    | 0.58    | 0.70    |
| 80.8-----                         | 380        | 0.48                                         | 0.66    | 0.64    | 0.76    |
| 80.8-----                         | 410        | 0.60                                         | 0.72    | 1.65    | N.d.    |
| 80.8-----                         | 440        | 0.66                                         | 1.80    | N.d.    | N.d.    |

N.d.—Not determined.

The above data show several interesting features of the X-PTHF materials as impact-improvers. Firstly, X-PTHF

## 12

of 80.8% or 86.6%/wt. gel content are not satisfactory since a mixing time as long as 10-15 minutes at 440° F. is not practical. Secondly, conversion of a very low molecular weight PTHF ( $\eta=1.1$ ), which per se is too low in molecular weight to produce high impact blends, to a corresponding highly gelled X-PTHF converts the material to an excellent impact improver. The latter material, however, produces blends of lesser thermal stability than the X-PTHF derived from a higher molecular weight PTHF parent. The X-PTHF derived from the PTHF parent of  $\eta=3.8$  exhibits very significantly improved thermal stability, high impact retention and broad processing latitude. The latter blends tenaciously retain their impact strength even after milling for 30 minutes at 335°-380° F. and after as much as 10 minutes at 410-440° F. Blends of polyvinyl chloride and the 1010 X 43 type material similar to those of Example IV begin to lose impact strength after 16 or 17 minutes at 380° F. and have essentially completely lost their impact strength in 16 minutes at 410° F. or after 10 minutes at 440° F. The PVC/X-PTHF blends such as those of this example have exceptionally wide processing latitude and great thermal stability. The blends containing X-PTHF are adapted to processing at the highest temperatures and in processing machines exhibiting appreciable hold-up of the stock under the highest processing temperatures.

## EXAMPLE VII

In this example, the use of auxiliary processing aids is investigated to show whether such are necessary and whether PTHF is compatible with the more common materials used as processing aids and/or lubricants. In this series of experiments four duplicate blends are prepared each containing 10 PHR of PTHF ( $\eta=3.22$ ) and the Izod impact values reported are obtained by averaging the four values. The data are as follows:

| Sample No. | Polyvinyl chloride base resin parts/wt. | Lubricant                  |           | TiO <sub>2</sub> parts/wt. | Type                             | Processing aid | Stabilizer* parts/wt. | Izod, ft./lbs./in. | Notes            |
|------------|-----------------------------------------|----------------------------|-----------|----------------------------|----------------------------------|----------------|-----------------------|--------------------|------------------|
|            |                                         | Type                       | Parts/wt. |                            |                                  |                |                       |                    |                  |
| 909A-----  | 100                                     | Cadmium stearate           | 2         | 5                          | Styrene-acrylonitrile copolymer. | 3              | 3                     | 10                 | 12.25 Good bank. |
| 909B-----  | 100                                     | do                         | 2         | 5                          | Polyethylene <sup>1</sup>        | 1.0            | 3                     | 10                 | 15.56 Do.        |
| 909C-----  | 100                                     | do                         | 2         | 5                          | Polypropylene <sup>2</sup>       | 1.0            | 3                     | 10                 | 16.27 Do.        |
| 909D-----  | 100                                     | Polyethylene <sup>1</sup>  | 1.0       | 5                          | Same as A                        | 3              | 3                     | 10                 | 4.82 Do.         |
| 909E-----  | 100                                     | Polypropylene <sup>2</sup> | 1.0       | 5                          | do                               | 3              | 3                     | 10                 | 9.10 Do.         |
| 909F-----  | 100                                     | Same as A                  | 2         | 5                          | None                             | 3              | 10                    | 1.61               |                  |

Chemical Corp.

<sup>2</sup> Amorphous polypropylene; low molecular weight.

It is clear that the good processing behavior of the PVC/PTHF blends of this invention is not due to any particular lubricant or processing aid. Likewise, the good impact resistance of such blends is not due to any particular lubricant/processing aid combination but rather from the PTHF additive. The improvement obtained through such auxiliary is normal.

55 We claim:

1. A resinous composition comprising for every 100 parts/wt. of a vinyl chloride base resin produced by the polymerization of a monovinylidene monomeric material containing at least 80% wt. of vinyl chloride from about 3 to about 20 parts/wt. of rubbery polymerized tetrahydrofuran exhibiting, in its nongelled condition, an intrinsic viscosity as determined in benzene 25° C. from about 1.5 up to 20 dl./gm.
2. Resinous composition according to claim 1 and further characterized by said base resin is polyvinyl chloride and the said polymerized tetrahydrofuran is uniformly dispersed in the said base resin.
3. A resinous composition according to claim 1 and further characterized by said polymerized tetrahydrofuran possessing a gel content in ethyl acetate of from about 25% to about 80%/wt.
4. A resinous composition according to claim 1 and further characterized by (1) said rubbery polymerized tetrahydrofuran being a substantially gel-free material having an intrinsic viscosity of from about 2 to about 15

and present in a proportion of from about 5 to about 10 parts/wt. and (2) said rubbery polymerized tetrahydrofuran is uniformly dispersed in and thoroughly fluxed with said base resin.

5. A resinous composition according to claim 1 where-  
in the said base resin is polyvinyl chloride, the said poly-  
merized tetrahydrofuran is substantially gel-free material  
having an intrinsic viscosity as defined of between about  
2 and about 4 dl./gm., and is present in a proportion of  
from about 5 to about 15 parts/wt., and said composition  
has been blended under high mechanical shear at a tem-  
perature of from about 350° to about 440° F.

6. A resinous composition comprising for every 100  
parts by weight of a polyvinyl chloride base resin from  
about 7 to about 15 parts/wt. of a polymerized tetrahy-  
drofuran containing from about 25% to about 75%/wt.  
of ethyl acetate insoluble gel, said gel-containing poly-  
merized tetrahydrofuran being derived by mixing a low  
gel polymerized tetrahydrofuran having an intrinsic viscos-  
ity as determined in benzene at 25° C. from about 1.0 to  
about 6.0 dl./gm. with a peroxide and sulfur and heat-

ing at a temperature of from about 75° to about 160° C.  
to generate therein the desired proportion of gel within  
the range specified.

7. A resinous composition according to claim 1 and  
further characterized by containing from about 0.2% to  
about 3%/wt. based on said polymerized tetrahydrofuran  
of a rubber antioxidant.

#### References Cited

##### UNITED STATES PATENTS

3,463,834 8/1969 Dreyfuss ----- 260—899

##### FOREIGN PATENTS

928,799 6/1963 Great Britain.

MURRAY TILLMAN, Primary Examiner

C. J. SECCURO, Assistant Examiner

##### U.S. CL. X.R.

260—41, 45.75, 49.95